



US005209807A

# United States Patent [19]

Fry

[11] Patent Number: 5,209,807  
[45] Date of Patent: May 11, 1993

[54] PAPERMAKERS FABRIC FOR CORRUGATION MACHINES

[75] Inventor: Ted Fry, Summerville, S.C.

[73] Assignee: Asten Group, Inc., Charleston, S.C.

[21] Appl. No.: 733,319

[22] Filed: Jul. 22, 1991

Related U.S. Application Data

[63] Continuation of Ser. No. 351,717, May 15, 1989, Pat. No. 5,050,646.

[51] Int. Cl.<sup>5</sup> B31F 5/00; D03D 11/00

[52] U.S. Cl. 156/470; 139/383 A; 139/408; 428/229; 428/225; 428/257

[58] Field of Search 156/470; 139/408, 383 A; 428/234, 225, 227, 229, 257

[56] References Cited

U.S. PATENT DOCUMENTS

- 4,169,007 9/1979 Pray 156/210 X  
4,174,739 11/1979 Raser et al. 139/408 X  
4,224,372 9/1980 Romanski 139/383 A X  
4,239,065 12/1980 Trokhan 139/383 A X

4,403,632 9/1983 Romanski et al. 139/383 A  
4,589,944 5/1986 Torti et al. 156/470 X  
4,935,082 6/1990 Bennett et al. 156/470

OTHER PUBLICATIONS

Scandia Corrugator Belt analysis sheet & drawing (2pgs.) Aug. 12, 1987.

Muhlen Sohn Aqua Pull Corrugator Belt analysis sheet & drawing (2pgs.) Mar. 3, 1988.

Asten J1338R Corrugator Belt analysis sheet (1pg.) Sep. 14, 1988.

Primary Examiner—Caleb Weston

Assistant Examiner—Michele K. Yoder

Attorney, Agent, or Firm—Volpe & Koenig

[57] ABSTRACT

A corrugation machine includes a woven papermakers fabric. The fabric has at least four layers of bulky yarns interwoven with monofilament yarns. The yarns and weave patterns are selected such that the fabric has a caliper of at least 0.2 inches, a weight of between 10 to 15 ounces per square foot and a permeability of at least 25 CFM.

4 Claims, 6 Drawing Sheets





FIG. 1

FIG. 2a  
PRIOR ARTFIG. 2b  
PRIOR ART



FIG. 4a



FIG. 4

FIG. 5a



FIG. 5b



FIG. 5c



FIG. 5d



FIG. 6a



四

## PAPERMAKERS FABRIC FOR CORRUGATION MACHINES

This is a continuation of U.S. patent application Ser. No. 07/351,717, filed May 15, 1989, now U.S. Pat. No. 5,050,646.

This invention relates to papermaking and more particularly to fabrics for use in papermaking machines which make corrugated paper products.

### BACKGROUND OF THE INVENTION

Generally a papermaking machine comprises a forming section, a press section and a dryer section. Papermakers fabrics transport an aqueous paper web through the machine to produce a paper product. Each of the three sections of the papermaking machine has its own unique characteristics and requirements. Accordingly, papermakers fabrics are specifically designed for each section of the papermaking machine such as forming fabrics for the forming section, wet press felts for the press section and dryer fabrics for the dryer section.

After a paper sheet is made by the conventional forming, pressing and drying operations, additional papermaking equipment can be used to manufacture corrugated material such as corrugated cardboard. As in the preliminary papermaking steps, a papermakers fabric is employed to transport the paper product during its manufacture. A corrugation machine combines separate paper sheets with an adhesive to form the corrugated paper product. As with other papermaking operations, the corrugation machine has its own unique demands on the performance of the papermakers fabric which transports the paper products therethrough.

Conventionally, corrugator belts, i.e. papermakers fabrics for corrugation machine, comprising a base fabric having one or more batts needed thereto have been utilized for the corrugation processing. Attempts have been made to utilize woven fabrics without batts as corrugation belts. For example, corrugator belts have been made having a woven fabric comprised entirely of spun polyester and polyester multifilament yarns in a three ply/three warp weave construction. Such fabrics are characterized by their relatively high weight, on the order of 20.59 oz./sq. ft., and low permeability, on the order of 4 CFM. (CFM as used herein means cubic feet per minute per square foot of fabric at  $\frac{1}{2}$  inch water pressure drop.)

At least one attempt has been made to provide a lightweight, high permeability fabric by constructing a  $4\frac{1}{2}$  ply fabric with monofilament polyester warp yarns and a combination of monofilament polyester, spun polyester and spun acrylic filling yarn layers. Although such fabric was relatively lightweight, on the order of 9.38 oz./sq. ft., and had relatively high permeability, on the order of 19 CFM, the caliper of the fabric was only 0.161 inches and the fabric had a relatively high moisture absorption characteristic.

It is desirable to provide a papermakers fabric for corrugation papermaking equipment which is relatively lightweight and permeable and which has a sufficient caliper to provide the fabric thickness desirable for processing associated with corrugation.

### SUMMARY AND OBJECTS OF THE INVENTION

A corrugation machine is provided with a woven papermakers fabric. The fabric comprises a system of

monofilament warp yarns interwoven with multiple layers of bulky yarns and monofilament yarns. The fabric has at least four layers of bulky yarns and at least three intermediate layers of monofilament yarns. At least two of the bulky yarn layers and one monofilament layer are disposed between two of the monofilament yarn layers. The yarns and weave patterns are selected such that the fabric has a caliper of at least 0.2 inches, a weight of between 10 to 15 ounces per square foot and a permeability of at least 25 CFM.

An object of the invention is to provide a corrugator belt having at least four layers of bulky yarns which are interwoven with monofilament yarns and, in particular, to provide at least three intermediate layers of monofilament filling yarns to provide a uniform structural network upon which top and bottom bulky yarn layers are woven.

The further object of the present invention is to provide a corrugator belt having a caliper of between 0.2 and 0.3 inches, a permeability between 25-50 CFM and a weight of about 12 ounces per square foot.

Other objects and advantages of the present invention will become apparent from following description of a presently preferred embodiment.

### BRIEF DESCRIPTION OF THE DRAWINGS

FIG. 1 is a schematic view of a portion of a corrugator machine:

FIGS. 2a-b are schematic diagrams of the weave structure of a prior art corrugator belt;

FIGS. 3a-b are schematic diagrams of the weave structure of a corrugator belt made in accordance with the teachings of the present invention;

FIGS. 4a-b are schematic diagrams of the weave structure of a first alternate embodiment of a corrugator belt made in accordance with the teachings of the present invention;

FIGS. 5a-d are schematic diagrams of the weave structure of a second alternate embodiment of a corrugator belt made in accordance with the teachings of the present invention; and

FIGS. 6a-b are schematic diagrams of the weave structure of a third alternate embodiment of a corrugator belt made in accordance with the teachings of the present invention.

### DETAILED DESCRIPTION OF PREFERRED EMBODIMENT

Referring to FIG. 1 there is shown a portion of a corrugator machine 10 having corrugator belts 12 and 14 which transport a corrugated paper product 15. The corrugated paper product comprises a top liner layer 15a, and intermediate corrugated layer 15b, and a bottom layer 15c to which an adhesive has been applied to maintain the corrugated structure of the final corrugated paper product such as corrugated cardboard. The separate layers 15a, 15b, 15c having adhesive applied therebetween are brought together at one end of the corrugator machine and transported by corrugator belt 12 across a series of hot plates 16 to dry and/or cure the adhesive which bonds the paper layers together.

The corrugator machine 10 includes a plurality of weighted rollers 17 and air plenums 18 which apply pressure to one surface of the fabric 12 so that the fabric transports the paper product 15 across the hot plates 16 under a selected amount of pressure. After passing over the series of hot plates 16 the corrugator belt 12 carries the paper product 15 between itself and the second

corrugator belt 14 which serves to maintain the speed of the process operation and to cool the paper product 15.

After exiting the corrugator belts 12, 14, the paper product 15 is cut and/or stacked as desired for the corrugator paper product being produced. The main corrugator belt 12 may then be subject to a shower mechanism 19 which cleans the fabric 12 as it runs.

With reference to FIGS. 2a-b, there is shown the weave structure of a prior art attempt to provide a woven papermakers fabric to serve as a corrugator belt. The fabric 20 comprises a bottom layer of spun polyester yarns 21, an intermediate and top layer spun acrylic yarns 22, 23 and two intermediate layers of monofilament yarns 24, 25. The filling yarn layers 21-25 are interwoven with a system of warp yarns 26. Analysis of one such fabric revealed warp yarns comprised of 0.020 inches polyester yarns woven 85 ends per inch and filling yarn layers totaling 56 picks per inch; the fabric having a caliper of approximately 0.161 inches, a permeability of about 19 CFM, and a weight of about 9.38 ounces per square foot. Although the sampled fabric was lightweight and had a relatively high permeability, its relatively thin caliper is potentially problematic for a corrugator belt and it exhibited a high moisture retention characteristic.

Referring to FIGS. 3a-b there is shown the weave diagram for a papermakers fabric 30 made in accordance with the teachings of the present invention. Unlike the prior art, the present invention comprises at least four layers of bulky yarns 31, 32, 33, 34. In addition, at least three layers 35, 36, 37 of intermediate monofilament filling yarns are provided to provide structural integrity and fabric stability to the thicker woven fabric.

The sundry filling layers 31-37 are disposed such that the fabric has a top layer 31 and a bottom layer 34 of bulky yarns. The intermediate layers of the fabric are disposed such that at least two layers 32, 33 of bulky yarns and one layer 36 of monofilament yarns are disposed between two layers 35, 37 of monofilament yarns.

The filling layers are interwoven with a system 38 of monofilament warp yarns which are preferably polyester yarns having a diameter of about 0.020 inches. The interweaving of the monofilament warp yarns 38 with the monofilament filling yarn layers 35, 36, 37 provides a stable fabric structure which maintains the position of the bulky yarns 31, 32, 33, 34 and the overall caliper of the fabric.

With respect to FIGS. 3a-b, there is shown a single layer 36 of monofilament yarns disposed between the interior two layers 32, 33 of bulky yarns. The system 38 of warp yarns is divided such that half of the monofilament warp yarns interweave with the top bulky yarn layer 31 and all three monofilament filling layers 35, 36, 37 and the other half of the monofilament warp yarns 55 interweave with the bottom bulky yarn layer 34 and all three monofilament filling layers 35, 36, 37.

As shown in FIGS. 3a-b, the system 38 of warp yarns is a 16-harness warp system. Yarns of warp system 38 are labelled 38a-p to indicate the sequence of weaving of the warp yarn harness. Preferably these yarns are polyester monofilament yarns having a diameter of 0.20 inches. Top and bottom filling yarn layers 31, 34 each contain eight yarns in their repeat labelled 31a-h, 34a-h respectively; the intermediate layers of filling yarns 32, 33, 35, 36, 37, each contain four yarns in their repeat which are labelled 32a-d, 33a-d, 35a-d, 36a-d, 37a-d, respectively.

Warp yarns 38a, 38c, 38e, 38g, 38i, 38k, 38m, 38o, each interweave under a separate bulky yarn in the repeat of bottom layer 34 and with the interior layers of the fabric. Since each of those warp yarns weaves under a single yarn of the bottom layer wft yarns 34, those warp yarns define knuckles on the bottom surface of the fabric. For example, yarn 38a weaves between yarns 36a and 37a, between yarns 31a and 34a, under yarn 33a, between yarns 31b and 34b, under yarn 37b, under yarn 34c, under yarn 33b, between yarns 31d and 34d, between yarns 36c and 37c, between yarns 31e and 34e, between yarns 32c and 33c, between yarns 31f and 34f, over yarn 35d, between yarns 31g and 34g, between yarns 32d and 33d, and between yarns 31h and 34h, whereafter the pattern is repeated. In a similar fashion warp yarn 38c interweaves with bottom layer yarn 34f; warp yarn 38m interweaves with bottom layer yarn 34e, and warp yarn 38i interweaves with bottom layer yarn 34g.

Warp yarn 38c interweaves with bottom layer 34f; warp yarn 38g interweaves with bottom layer yarn 34d, warp yarn 38k interweaves with bottom layer yarn 34b, and warp yarn 38o interweaves with bottom layer yarn 34h in a similar but slightly different manner. For example, warp yarn 38g weaves over yarn 35a, between yarns 31a and 34a, between yarns 32a and 33a, between yarns 31b and 34b, between yarns 36b and 37b, between yarns 31c and 34c, under yarn 33b, under yarn 34d, under yarn 37c, between yarns 31e and 34e, under yarn 33c, between yarns 31f and 34f, between yarns 36d and 37d, between yarns 31g and 34g, between yarns 32d and 33d, between yarns 31h and 34h and thereafter repeats.

Warp yarns 38b, 38d, 38f, 38h, 38j, 38l, 38n, and 38p interweave over top layer bulky yarns 31a, 31d, 31g, 31b, 31e, 31h, 31c, and 31f, respectively, in a mirror image of the warp yarns which weave under the bottom layer 34 of bulky filling yarns as described above. Accordingly, warp yarns 38b, 38d, 38f, 38h, 38j, 38l, 38n and 38p define knuckles on the top surface of the fabric.

Preferably the fabric is woven flat and seamed when installed on a corrugator machine. The seam is preferably made by clinching large metallic hooks in both ends of the fabric and joining the hooks with a plastic coated solid core pintle.

Preferably polyester spun yarn made from 15 denier fibers are used for the bulky yarns. This, in cooperation with the weave, results in a relatively high permeability of the entire fabric. For example, a trial fabric was woven in accordance with the prior art weave structure depicted in FIG. 1 having a warp system woven at 60 yarns per inch interwoven with filling yarns totaling 52.5 picks per inch. The bulky yarns were 400 yard per pound polyester spun yarns made from 6 denier fibers. That trial fabric weighed approximately 10.2 ounces per square foot, had a permeability of about 15 CFM and a caliper of about 0.185 inches.

In contrast, a test sample of a fabric was woven in accordance with the weave structure depicted in FIG. 3a-b, with 400 yard per pound polyester yarns made from 15 denier fibers utilized as bulky yarns for the filling layers 31-35, 0.032 inch diameter polyester monofilament filling yarns, and 0.020 inch diameter polyester monofilament warp yarns. That sample was woven approximately 60 warp ends per inch and 65 picks per inch, resulting in a fabric having a weight of approximately 12 ounces per square foot, a permeability of approximately 27 CFM and a caliper of about 0.21 inches. Use of polyester monofilament is preferred to

minimize moisture retention and maximize dimensional stability. Use of polyester bulky yarn is preferred to minimize moisture retention.

Increased fabric stability and caliper is provided by the alternative embodiments depicted in FIGS. 4a-b, 5a-d, and 6a-b. In each of those embodiments four monofilament filling layers are provided. The interior most two layers are substantially coplanar with the interior bulky yarn layers. Such structure provides increased caliper while maintaining the other desirable characteristics of the corrugator fabric.

With reference to FIGS. 4a-b, there is shown a 16-harness monofilament warp system 41 which selectively interweaves in a repeat pattern with four layers of bulky yarns 42, 43, 44, 45 and four layers of monofilament yarns 46, 47, 48, 49.

As with the preferred embodiment, half of the monofilament warp yarns of the fabric shown in FIGS. 4a-b, interweave with the top bulky yarn filling layer 42 and three of the monofilament filling layers 46, 47, 48 and the other half of the warp yarns weave with the bottom bulky yarn filling layer 45 and three of the monofilament filling layers 47, 48, 49.

As shown in FIG. 4a-b, the system 41 of warp yarns is a 16-harness warp system. Yarns of warp system 41 are labelled 41a-p to indicate the sequence of weaving of the warp yarn harness. Preferably these yarns are polyester monofilament yarns having a diameter of 0.20 inches. Top and bottom filling yarn layers 42, 45 each contain eight yarns in their repeat labelled 42a-h, 45a-h respectively; the intermediate layers of filling yarns 43, 44, 46, 47, 48, 49, each contain four yarns in their repeat which are labelled 43a-d, 44a-d, 46a-d, 47a-d, 48a-d, 49a-d, respectively.

Warp yarns 41a, 41c, 41e, 41g, 41i, 41k, 41m, 41o, each interweave under a separate bulky yarn in the repeat of bottom layer 45 and with the interior layers of the fabric. For example, yarn 41a weaves over yarn 47a, between yarns 42a and 45a, between yarns 43a and 44a, between yarns 42b and 45b, between yarns 47b and 48b, between yarns 42c and 45c, under yarn 44b, between yarns 42d and 45d, under yarn 49c, under yarn 45e, under yarn 44c, between yarns 42f and 45f, between yarns 48d and 49d, between yarns 42g and 45g, between yarns 43d and 44d, and between yarns 42h and 45h whereafter the pattern is repeated. In a similar fashion warp yarn 41c interweaves with bottom layer yarn 45h; warp yarn 41e interweaves with bottom layer yarn 45g, and warp yarn 41g interweaves with bottom layer yarn 45b.

Warp yarns 41i interweaves with bottom layer 45f, warp yarn 41k interweaves with bottom layer yarn 45c, warp yarn 41m interweaves with bottom layer yarn 45a, and warp yarn 41o interweaves with bottom layer yarn 45d in a similar but slightly different manner. For example, warp yarn 41o weaves over yarn 47a between yarns 42a and 45a, between yarns 43a and 44a, between yarns 42b and 45b, between yarns 48b and 49b, between yarns 42c and 45c, under yarn 44b, under yarn 45d, under yarn 49c, between yarns 42e and 45e, under yarn 44c, between yarns 42f and 45f, between yarns 47d and 48d, between yarns 42g and 45g, between yarns 43d and 44d, between yarns 42h and 45h and thereafter repeats.

Warp yarns 41b, 41d, 41f, 41h, 41j, 41l, 41n, and 41p interweave over top layer bulky yarns 42b, 42g, 42d, 42a, 42e, 42h, 42f, and 42c, respectively, in a mirror image of the warp yarns which weave under the bottom layer 45 of bulky filling yarns as described above.

Where four layers of monofilament filling yarns are desired, the interweaving system of monofilament warp yarns may include selected warp yarns which interweave only with intermediate filling yarn layers. Such weaves provides additional structural integrity to enhance the stability of the fabric.

With reference to FIGS. 5a-d, there is shown a 16-harness monofilament warp system 51 which selectively interweaves in a repeat pattern with four layers of bulky yarns 52, 53, 54, 55 and four layers of monofilament yarns 56, 57, 58, 59. In this embodiment half of the warp yarns interweave entirely in the interior fabric.

As shown in FIGS. 5a-d, the system 51 of warp yarns is a 16-harness warp system. Yarns of warp system 51 are labelled 51a-p to indicate the sequence of weaving of the warp yarn harness. Preferably these yarns are polyester monofilament yarns having a diameter of 0.20 inches. Top and bottom filling yarn layers 52, 55 each contain eight yarns in their repeat labelled 52a-h, 55a-h respectively; the intermediate layers of filling yarns 53, 54, 56, 57, 58, 59, each contain four yarns in their repeat which are labelled 53a-d, 54a-d, 56a-d, 57a-d, 58a-d, 59a-d, respectively.

Warp yarns 51a, 51c, 51e, 51g, 51i, 51k, 51m, 51o, each interweave over a separate bulky yarn in the repeat of top layer 52 and under a separate bulky yarn in the repeat of bottom layer 55. For example, yarn 51a weaves between yarn 57a and 58a, between yarns 52a and 55a, over yarn 53a, over yarn 52b, over yarn 56b, between yarns 52c and 55c, over yarn 53b, between yarns 52d and 55d, between yarns 57c and 58c, between yarns 52e and 55e, under yarn 54c, between yarns 52f and 55f, under yarn 59d, under yarn 55g, under yarn 54d, and between yarns 52h and 55h whereafter the pattern is repeated. In a similar fashion warp yarn 51c interweaves with top and bottom layer yarns 52f and 55c; warp yarn 51e interweaves with top and bottom layer yarns 52h and 55e; warp yarn 51g interweaves with top and bottom layer yarns 52d and 55a; warp yarn 51i interweaves with top and bottom layers yarns 52a and 55d, warp yarn 51k interweaves with top and bottom layer yarns 52e and 55h, warp yarn 51m interweaves with top and bottom layer yarns 52c and 55f; and warp yarn 51o interweaves with top and bottom layer yarns 52g and 55b.

Warp yarns 51b, 51d, 51f, 51h, 51j, 51l, 51n, and 51p interweave entirely with the intermediate filling layers 53, 54, 56, 57, 58 and 59. For example, warp yarn 51b weaves over yarn 56a, between yarns 52a and 55a, over yarn 53a, between yarns 52b and 55b, between yarns 56b and 57b, between yarns 52c and 55c, between yarns 53b and 54b, between yarns 52d and 55d, between yarns 58c and 59c, between yarns 52e and 55e, between yarns 53c and 54c, between yarns 52f and 55f, between yarns 56d and 57d, between yarns 52g and 55g, over yarn 53d, between yarns 52h and 55h and thereafter repeats.

With reference to FIGS. 6a-b, there is shown a 14-harness monofilament warp system 61 which selectively interweaves in a repeat pattern with four layers of bulky yarns 62, 63, 64, 65 and four layers of monofilament yarns 66, 67, 68, 69. In this embodiment, six of the fourteen yarns interweave entirely in the interior fabric.

As shown in FIGS. 6b, the system 61 of warp yarns is a 14-harness warp system. Yarns of warp system 61 are labelled 61a-n to indicate the sequence of weaving of the warp yarn harness. Preferably these yarns are polyester monofilament yarns having a diameter of 0.20 inches. Top and bottom filling yarn layers 62, 65 each

contain eight yarns in their repeat labelled 62a-h, 65a-h respectively; the intermediate layers of filling yarns 63, 64, 66, 67, 68, 69, each contain four yarns in their repeat which are labelled 63a-d, 64a-d, 66a-d, 67a-d, 68a-d, 69a-d, respectively.

Warp yarns 61a, 61e, 61j, 61k, each interweave over two separate bulky yarns in the repeat of top layer 62 and with two of the interior monofilament 66, 67 layers of the fabric. For example, warp yarn 61a weaves over yarn 66a, between yarns 62a and 65a, over yarn 63a, between yarns 62b and 65b, between yarns 67b and 68b, between yarns 62c and 65c, over yarn 63b, over yarn 62d, over yarn 66c, between yarns 62e and 65e, over yarn 63c, between yarns 62f and 65f, between yarns 67d and 68d, between yarns 62g and 65g, over yarn 63d, and over yarn 62h whereafter the pattern is repeated. In a similar fashion warp yarn 61e interweaves with top layer yarns 62b and 62f.

Warp yarns 61j interweaves with top layer yarns 62a and 62e, and warp yarn 61k interweaves with top layer yarns 62c and 62g, in a similar but slightly different manner. For example, warp yarn 61j weaves over yarn 66a, over yarn 62a, over yarn 63a, between yarns 62b and 65b, between yarns 67b and 68b, between yarns 62c and 65c, over yarn 63b, between yarns 62d and 65d, over yarn 66c, over yarn 62e, over yarn 63c, between yarns 62f and 65f, between yarns 67d and 68d, between yarns 62g and 65g, over yarn 63d, between yarns 62h and 65h and thereafter repeats.

Warp yarns 61c, 61h, 61i, 61l interweave under bottom layer bulky yarn pairs 65d and 65h, 65b and 65f, 65a and 65e, 65c and 65g, respectively, in a mirror image of the warp yarns which weave over the top layer 62 of bulky filling yarns as described above.

Warp yarns 61b, 61d, 61f, 61g, 61m, and 61n interweave entirely with the intermediate filling layers, each interweaving with two of the monofilament layers 66, 67, 68 and 69. For example, warp yarn 61b weaves between yarns 67a and 68a, between yarns 62a and 65a, over yarn 63a, between yarns 62b and 65b, over yarn 66b, between yarns 62c and 65c, over yarn 63b, between yarns 62d and 65d, between yarns 67c and 68c, between yarns 62e and 65e, over yarn 63c, between yarns 62f and 65f, over yarn 66d, between yarns 62g and 65g, over yarn 63d, between yarns 62h and 65h and thereafter repeats. Yarn 61m weaves in a mirror image with monofilament layers 66 and 67 between bulky filling yarn layers 62 and 63. Similarly, yarns 61f and 61g interweave with monofilament layers 67 and 68 between bulky filling yarn layers 63 and 64 and yarns 61d and 61n interweave with monofilament layers 68 and 69 between bulky filling yarn layers 64 and 65.

These latter two weave structures, FIGS. 5a-d and 6a-b, additionally help to maintain the stability and the caliper of the overall fabric by maintaining the relative vertical alignment and spacing of the yarns of the mono-

filament filling layers. Although several specific warp harness weaves are disclosed, other configurations of monofilament warp systems could be used to interweave the multiple layers of filling yarns.

5 What I claim is:

1. A corrugator belt comprising a system of monofilament warp yarns interwoven with a top layer of bulky filling yarns, a bottom layer of bulky filling yarns and at least two intermediate layers of bulky filling yarns in a repeat pattern with selected monofilament warp yarns weaving knuckles over the top layer of filling yarns and with selected monofilament warp yarns weaving knuckles under the bottom layer of filling yarns such that the top layer of bulky filling yarns in conjunction with monofilament warp yarn knuckles define the top surface of the belt and such that the bottom layer of the bulky filling yarns in conjunction with the monofilament warp yarn knuckles define the bottom surface of the belt.

10 2. A corrugator belt according to claim 1 wherein said system of monofilament warp yarns is interwoven with said bulky filling yarns such that the belt has a substantially uniform caliper of at least 0.2 inches, a substantially uniform permeability of at least 25 CFM and a substantially uniform weight of less than 15 ounces per square foot.

15 3. A corrugator apparatus for manufacturing corrugated paper products, the apparatus having a series of heat element means spaced from and associated with pressure application means to facilitate the processing of the corrugated paper product, a papermakers fabric which traverses between said heat element means and said pressure application means to transport the paper product across the heat element means, and wherein the papermakers fabric comprises a system of monofilament warp yarns interwoven with a top layer of bulky filling yarns, a bottom layer of bulky filling yarns and at least two intermediate layers of bulky filling yarns in a repeat pattern with selected monofilament warp yarns weaving knuckles over the top layer of filling yarns and with selected monofilament warp yarns weaving knuckles under the bottom layer of filling yarns such that the top layer of bulky filling yarns in conjunction with monofilament warp yarn knuckles define the top surface of the fabric and such that the bottom layer of the bulky filling yarns in conjunction with the monofilament warp yarn knuckles define the bottom surface of the fabric.

20 4. A corrugator apparatus according to claim 3 wherein said system of monofilament warp yarns is interwoven with said bulky filling yarns such that the fabric has a substantially uniform caliper of at least 0.2 inches, a substantially uniform permeability of at least 25 CFM and a substantially uniform weight of less than 15 ounces per square foot.

\* \* \* \* \*

UNITED STATES PATENT AND TRADEMARK OFFICE  
CERTIFICATE OF CORRECTION

PATENT NO. : 5,209,807  
DATED : May 11, 1993  
INVENTOR(S) : Ted Fry

It is certified that error appears in the above-identified patent and that said Letters Patent is hereby corrected as shown below:

At column 4, line 5, delete "wft" and insert therefor --  
weft --.

IN THE CLAIMS

In claim 3, at column 8, line 35, delete "and".

Signed and Sealed this

Eleventh Day of January, 1994

Attest:



BRUCE LEHMAN

Attesting Officer

Commissioner of Patents and Trademarks